

# United States Patent Office

2,944,890

Patented July 12, 1960

1

2,944,890

## ALUMINUM BRONZE ALLOY HAVING IMPROVED WEAR RESISTANCE BY THE ADDITION OF COBALT AND CHROMIUM

John F. Klement, Milwaukee, Wis., assignor to Ampco Metal, Inc., Milwaukee, Wis., a corporation of Wisconsin

No Drawing. Filed Jan. 22, 1958, Ser. No. 710,410

5 Claims. (Cl. 75—162)

This invention relates to an aluminum bronze alloy and more particularly to an aluminum bronze alloy having improved toughness and wear resistance.

Aluminum bronze alloys have for years been used as dies for forming and drawing operations for a large group of sheet and plate alloys, such as stainless steel, aluminum, nickel, titanium, mild steel and some copper base alloys. Aluminum bronze alloys used in die applications possess the properties of good corrosion resistance, wear resistance and non-galling against many wrought materials.

The aluminum bronze alloys which in the past have shown the optimum properties for deep drawing dies are those that contain approximately 14% aluminum, a small amount of iron and the balance copper. An alloy of this type has good corrosion resistance and non-galling properties. However, under heavy use in die application, it wears undesirably fast so that close dimensional tolerances cannot be maintained because of the wear that occurs on the die surface.

The present invention is directed to an aluminum bronze alloy which has the corrosion resistance and the non-galling properties characteristic of aluminum bronze alloys but has greatly improved wear resistance and toughness.

The aluminum bronze alloy of the invention has high uniform hardness, good toughness and excellent wear resistance. This is accomplished by the addition of small amounts of cobalt and chromium to the alloy which substantially reduces the tendency of the alloy to form the eutectoid. The addition of cobalt and chromium also makes the alloy more homogeneous in the distribution of the metallurgical phases and compounds during solidification and heat treatment and also promotes uniform controlled grain size.

Furthermore, the alloy, particularly at the lower end of the chromium range, has a finer and rounder particle size than the ordinary aluminum bronze alloy which results in better machinability.

The alloy of the invention has the following general composition by weight:

|          | Percent   |
|----------|-----------|
| Aluminum | 13.0-20.0 |
| Iron     | 1.0- 8.0  |
| Cobalt   | 0.5- 5.0  |
| Chromium | 0.5- 3.0  |
| Copper   | Balance   |

This alloy has a tensile strength of about 65,000 to 105,000 p.s.i., a yield strength of 65,000 to 80,000 p.s.i., an elongation in two inches of up to 2.5% and a Rockwell C hardness in the range of 25 to 55.

A specific illustration of the composition of the alloy falling within the above range is as follows in weight percent:

|          | Percent |
|----------|---------|
| Aluminum | 15.10   |
| Iron     | 5.01    |
| Cobalt   | 3.18    |
| Chromium | 1.50    |
| Copper   | 73.93   |

2

The above alloy can be cast either statically or centrifugally to produce a fine grained tough structure having, in the chilled cast state, a tensile strength of 100,000 p.s.i., a yield strength of 75,000 p.s.i., an elongation in two inches of 1.5% and a Rockwell C hardness of 40.

The alloy of the invention has greatly improved wear resistance over that of an ordinary aluminum bronze alloy and this increase in wear resistance is most significant since the hardness of the alloy is substantially the same as the hardness of an aluminum bronze alloy having similar proportions of aluminum and iron but not containing the cobalt and chromium. For example, the wear resistance of the present alloy is about 50% to 80% better than the conventional aluminum bronze alloy, the toughness is 100% to 150% better, and the machinability, at the lower chromium contents, is about 100% better than the ordinary aluminum bronze alloy not containing the cobalt and chromium.

The metallographic structure of the alloy consists essentially of gamma two phase which is uniformly distributed in a matrix of beta. An intermediate compound composed of iron, aluminum, copper, cobalt and chromium exists in small particles of uniform size and shape. Because of the method of casting and the inoculant used, the intermetallic compound is uniformly distributed throughout the cast section.

In order to obtain optimum properties, the metals used for the alloy should be of high quality. Electrolytic or wrought fire refined copper, high purity aluminum, low carbon iron and high purity cobalt and chromium are preferred to be used. It has also been found that the best method of obtaining the desired uniformity in the alloy is by using a double melting procedure whereby a pre-alloy is made. The most satisfactory pre-alloy is one that has approximately 45% aluminum, 20% copper, 15% iron, 10% chromium and 10% cobalt.

The melting procedure employed in making the pre-alloy is such that some copper, along with the iron, chromium and cobalt, is placed into the crucible and melting begun. When the copper starts to melt, the iron and other additives are slowly dissolved into the copper during that period when aluminum is added to form an exothermic reaction which helps to dissolve the higher melting point cobalt and chromium additions. This prealloy is then cast into ingot form and is ready to use for the final alloy.

The final alloy is made by intermixing a predetermined percentage of the pre-alloy and copper. A deoxidizer is added to this alloy in the molten state in the furnace to purge the metal of oxides and soluble gases. These deoxidizers can include the compounds of boron, phosphorus, magnesium and lithium. Deoxidizers of the gas type can also be used. This can include volatile chlorides or any of the inert gases. The dry type deoxidizers are added in quantities of approximately 4 ounces per 100 pounds of metal, and the gas type deoxidizers are passed either through or over the molten metal for a period of five minutes. Removal of the oxide particles is of particular importance because of their abrasive and adverse effect on the wear-resistant properties of the alloy.

Alternately, instead of employing a pre-alloy, the chromium and cobalt can be added directly to a molten aluminum-iron-copper alloy.

To establish complete uniformity of the microstructure and hardness the alloy is heat treated at an elevated temperature in the temperature range of 1050° F. to 1400° F., such as about 1150° F. Small castings of simple shapes of this alloy can be placed directly into the heat treating furnace at temperature. Large massive castings or intricate shapes are preheated in the furnace at about 400° F. until the section reaches uniform temperature and then are heated directly to the elevated temperature.

The castings are held at a temperature in the range of 1050° F. to 1400° F. for one hour plus one-half hour per inch of section thickness greater than one inch, up to a maximum of two and one-half hours at temperature.

After the required soaking time at the elevated temperature, the alloy is cooled at a rate faster than about 20° F. per hour per one inch of section thickness. This rate is conveniently obtained by fan air cooling.

Internal stresses created within castings during machining or other finishing operations, during weldments or from metal overlays on base metals, are usually removed depending on the future application of the part. These stresses are removed by a stress relief heat treatment. The usual commercial aluminum bronze alloys cannot generally be stress relieved at a temperature in the range of 650° F. to 1050° F. due to eutectoid formation that occurs at this temperature range. Furthermore, a stress relief at temperatures above 1050° F. frequently causes distortions and further stresses in the usual commercial aluminum bronze alloy during the rapid cooling to room temperature. Stress relief at temperatures lower than 650° F. takes considerable time and often the most severe stresses remain.

In contrast to this, the alloy of the invention can be stress relieved within the temperature range of 650° F. to 1050° F. without excessive embrittlement due to the eutectoid structure. An optimum stress relief temperature for the present alloy, based on the severity of the internal stresses and geometry of the article, can be selected in the range of 650° F. to 1050° F. to obtain a reasonable holding time in the furnace, such as one to two hours per 2 inches of section, and to prevent distortions and micro stresses during cooling. The article is then cooled to room temperature.

The alloy can be used to produce articles for wear resistant applications in drawing and forming operations. The articles may take the form of deep drawing dies, hold down dies, wear guides, forming rolls, skids, slides, etc.

The alloy can also be extruded into weldrods or weld wire. The alloy in the form of coated or uncoated weldrod can be overlaid on a base metal by metal spraying or other welding methods, such as heli-arc, metal-arc, carbon-arc, etc. to obtain a corrosion resistant wear surface. The metal overlay can be given a stress relief treatment at temperatures in the range of 650° F. to 1150° F. and cooled to room temperature.

It has been found that the addition of cobalt and chromium to the copper-aluminum-iron alloys to be used as die materials greatly improves the toughness and wear resistance of the alloy and substantially reduces the tendency for eutectoid embrittlement. As the alloy of the invention will not form the embrittling eutectoid structure to any great extent, more alloying elements can be incorporated in the alloy for a given hardness to thereby obtain increased wear resistance.

Various modes of carrying out the invention are contemplated as being within the scope of the following claims particularly pointing out and distinctly claiming the subject matter which is regarded as the invention.

I claim:

1. An aluminum bronze alloy, consisting essentially of 13.0% to 20.0% aluminum, from 1.0% to 8.0% iron, from 0.50% to 5.0% cobalt, from 0.5% to 3.0% chromium and the balance being substantially copper, said alloy being characterized by having excellent corrosion resistance and having improved toughness and wear resistance.

2. An aluminum bronze alloy having improved wear resistance, toughness and machinability, consisting essentially of from 13.0% to 20.0% aluminum, 1.0% to 8.0% iron, 0.5% to 5.0% cobalt, 0.5% to 3.0% chromium and the balance substantially copper, said alloy being characterized by a tensile strength in the range of 65,000 to 105,000 p.s.i., a yield strength in the range of 65,000 to 80,000 p.s.i., an elongation in two inches of up to 2.5%, and a hardness in the range of 25 to 55 Rockwell C.

3. An aluminum bronze alloy having improved toughness and wear resistance, consisting essentially of 15.10% aluminum, 5.01% iron, 3.18% cobalt, 1.50% chromium and 73.93% copper.

4. A drawing die characterized by having excellent corrosion resistance, a hardness in the range of 25 to 55 Rockwell C. and improved wear resistance, said die being fabricated from an aluminum bronze alloy consisting essentially of 13% to 20% aluminum, from 1% to 8% iron, from 0.5% to 5% cobalt, from 1% to 3% chromium, and the balance being substantially copper.

5. An aluminum bronze welding electrode consisting essentially of 13% to 20% aluminum, from 1% to 8% iron, from 0.5% to 5% cobalt, from 1.0% to 3.0% chromium, and the balance being substantially copper.

#### References Cited in the file of this patent

#### UNITED STATES PATENTS

|           |              |               |
|-----------|--------------|---------------|
| 2,789,900 | Hannon       | Apr. 23, 1957 |
| 2,809,139 | Bloom et al. | Oct. 8, 1957  |
| 2,829,971 | Klement      | Apr. 8, 1958  |
| 2,829,972 | Klement      | Apr. 8, 1958  |
| 2,832,709 | Sendzimir    | Apr. 29, 1958 |

#### FOREIGN PATENTS

|         |               |               |
|---------|---------------|---------------|
| 537,404 | Great Britain | June 20, 1941 |
|---------|---------------|---------------|

#### OTHER REFERENCES

"Non-Ferrous Tubes in the Stress of Modern Conditions," Breckon et al., Metal Industry, August 1, 1958, pages 89-90.

Ellis: Copper and Copper Alloys (American Society for Metals, 1948), pages 162-170.

Aluminum Bronze (London: Copper Development Association, 1939), pages 45-50.